

1

3,139,325

PROCESS FOR THE PRODUCTION OF TITANIUM  
AND ZIRCONIUM HYDROGEN PEROXIDE  
PRODUCTS

Koji Takada, Shinjuku-ku, Tokyo, Japan, assignor to Toyo  
Kinzokukagaku Kabushikikaisha, Tokyo, Japan  
No Drawing. Filed Mar. 6, 1961, Ser. No. 93,326  
Claims priority, application Japan Jan. 28, 1961  
4 Claims. (Cl. 23—14)

The invention relates to a novel process for the production of titanium and zirconium compounds, for use in the formation of alloy coatings consisting of cadmium or zinc, on the one hand, and titanium or zirconium, on the other hand.

It has been already proposed by me to produce alloy coatings of the kind above referred to in such a way that a pertitanate and a perzirconate is dissolved in a conventional coating bath containing cadmium cyanide or zinc cyanide and the electrolysis is carried out with use of cadmium or zinc as anode.

The main object of the invention is to provide a novel process for the production of titanium and zirconium compound, especially adapted to add to the coating bath in the above proposed coating process.

Tetrahydroxide of titanium or zirconium can be obtained, when a solution of tetravalent salts of titanium or zirconium, such as, for instance, titanium tetrafluoride, zirconium tetrafluoride or the like, is subjected to a hydrolysis in the presence of an alkali. The thus obtained tetrahydroxides are variable in their chemical and physical properties, depending upon the temperature and other conditions during the hydrolysis to a substantial degree. Thus, there are a plurality of isomers of tetrahydroxides of titanium and zirconium. It is, therefore, the more specific object of the invention to provide a novel process for the production of such titanium or zirconium tetrahydroxide which easily reacts with hydrogen peroxide to form the corresponding addition product liable to solve stably in an alkaline solution and thereby to form the pertitanate or perzirconate. According to my profound experiments, salts of strong acids, such as, for instance, the fluorides, chlorides, sulphates and the like are preferably used as the above mentioned tetravalent salts of titanium or zirconium, while salts of weak acids are liable to be subjected to hydrolysis and thus to form an unwanted titanium or zirconium compounds such as oxy-compounds. On the other hand, solutions of tetravalent compounds of titanium or zirconium, if diluted, are susceptible to hydrolysis. It is thus preferable in the present process to employ concentrations of these solutions lying in the neighborhood of the saturation point.

According to the invention, the hydrolysis of tetravalent titanium and zirconium salt is carried out at a temperature lower than 10° C. In the course of the alkaline hydrolysis, the temperature of the hydrolyte increases substantially and if the reaction temperature should become higher than 10° C., the produced hydroxides would provide such chemically inactive acids as meta-titanic acid or meta-zirconic acid, which adversely affects the production of the desired stable addition compounds with hydrogen peroxide.

According to the invention, the hydrolysis is carried out under sufficient cooling to produce highly reactive hydroxides or ortho-titanic or ortho-zirconic acid, thus capable of producing stable addition compounds with hydrogen peroxide. When the thus produced hydroxides are brought into reaction with the equivalent quantity of hydrogen peroxide, a paste-like substance consisting of titanium or zirconium hydroxide-hydrogen peroxide addition compound is formed, as the case may be.

2

In the process according to the invention, 1-5% of sodium pyrophosphate is added in the above mentioned stage to the hydrogen peroxide, which measure constitutes a feature of the invention. It was now found that the pyrophosphate reacts with hydrogen peroxide to form the peroxide of sodium pyrophosphate, which serves for stabilization of the titanium compound.

The above mentioned additional compounds dissolve in an alkaline solution to form the peroxide of sodium pertitanate or perzirconate, as the case may be. The addition compounds are not only highly stable and persist for long intervals, but also dissolve stably in an alkaline coating bath containing cadmium or zinc, from which the desired alloy coating containing titanium or zirconium can be produced in the conventional way.

The invention can be more fully understood with reference to the following several examples:

*Example 1*

20 A saturated aqueous solution of titanium tetrafluoride was ice-cooled and kept at a temperature lower than 5° C. An equivalent quantity of caustic soda was added and the resulting mixture was permitted to hydrolyze. The thus produced precipitate was then filtered and mixed with an equivalent quantity of hydrogen peroxide (of 35% concentration) containing 5% of sodium pyrophosphate, thus forming titanium hydroxide-hydrogen peroxide addition compound, which is highly stable. This addition compound was then dissolved in a conventional cyanate bath containing cadmium or zinc, therefrom a titanium alloy coating was produced in the conventional way.

*Example 2*

35 A saturated aqueous solution of zirconium tetrachloride was ice-cooled and kept at 3° C., and then subjected to hydrolysis in the presence of ammonia and centrifuged. The thus separated precipitate is reacted with an equivalent quantity of hydrogen peroxide (of 35% concentration) containing 3% of sodium pyrophosphate, thus forming zirconium hydroxide-hydrogen peroxide addition compound. This compound together with the titanium additional compound obtained in Example 1, was dissolved in a conventional zinc cyanide and subjected to an electrolysis, thus obtaining a ternary alloy coating containing zinc, titanium and zirconium.

45 Although for the purpose of explaining the invention certain particular examples thereof have been disclosed, obvious modifications will occur to a person skilled in the art, and it is not desired to be limited to the exact details described.

50 What is claimed and desired to be secured by Letters Patent is:

1. Process for the production of titanium and zirconium addition products particularly suited to be added to a plating bath containing a cyanide selected from the group consisting of cadmium cyanide and zinc cyanide, said process comprising: preparing a substantially saturated aqueous solution of a salt of a tetravalent metal selected from the group consisting of titanium and zirconium, said salt being selected from the group consisting of the fluorides, chlorides and sulfates of said tetravalent metal; adding an alkali selected from the group consisting of alkali metal hydroxides and ammonium hydroxide to said aqueous salt solution while maintaining the solution and resulting products at a temperature below 10° C.; physically separating the thereby produced precipitated hydroxide from the remaining liquid; then reacting said hydroxide with a chemically equivalent quantity of hydrogen peroxide in the presence of between 1% and 5% by weight of sodium pyrophosphate based on the hydrogen peroxide; and recovering the metal hydroxide-hydrogen peroxide addition product, so produced.

2. The process of claim 1, where in the salt is titanium tetrafluoride.

3. The process of claim 1 wherein the salt is zirconium tetrachloride.

4. The process of claim 1 wherein the hydrolysis is carried out in the presence of caustic soda added to said aqueous salt solution.

References Cited in the file of this patent

UNITED STATES PATENTS

|           |            |               |
|-----------|------------|---------------|
| 1,624,162 | Boer ----- | Apr. 12, 1927 |
| 2,141,189 | Lind ----- | Dec. 27, 1938 |

10

2,150,060 Guttenberg et al ----- Mar. 7, 1939

2,333,444 Robinson ----- Nov. 2, 1943

OTHER REFERENCES

Mellor: Comprehensive Treatise on Inorganic and Theoretical Chemistry, Longmans, Green and Co., New York, 1927, vol. VII, pages 130 to 132.

Schumb et al.: Hydrogen Peroxide, Reinhold Publishing Corporation, New York, No. 128, pages 540 and 541 (1955).

Blumenthal: The Chemical Behavior of Zirconium, D. Van Nostrand Co., Inc., New York, 1958, pages 198-200.